

# UNITED STATES PATENT OFFICE.

MILTON C. WHITAKER, OF NEW YORK, N. Y., ASSIGNOR TO U. S. INDUSTRIAL ALCOHOL CO., A CORPORATION OF WEST VIRGINIA.

## ENGINE FUEL.

1,421,879.

Specification of Letters Patent.

Patented July 4, 1922.

No Drawing.

Application filed November 12, 1919. Serial No. 337,396.

To all whom it may concern:

Be it known that I, MILTON C. WHITAKER, a citizen of the United States, residing at New York city, in the county of New York and State of New York, have invented a certain new and useful Improvement in Engine Fuel, of which the following is a specification.

My invention relates particularly to fuels adapted to be used in burners or internal combustion engines generally.

The object of my invention is to provide an efficient fuel for such use, which contains a comparatively heavy hydrocarbon, but the constituents of which are such as to enable the fuels to be utilized if desired in the same manner as the light hydrocarbon fuels previously used for this purpose.

Another object of my invention is to provide motor fuels containing hydrocarbons from which the lower paraffine hydrocarbons above propane, up to and including heptane, are substantially absent.

Again, another object of my invention is to provide motor fuels containing in addition to the comparatively heavy hydrocarbon an ester but which is preferably a volatile ester.

Further objects of my invention will appear from the detailed description thereof contained hereinafter.

For example, in carrying out my invention, I may provide a motor fuel comprised of the following:

35 90 to 92 parts by volume of kerosene, 8 to 10 parts by volume of ethyl acetate.

The kerosene may be any light hydrocarbon distillate having a specific gravity heavier than 50° Bé. These are usually hydrocarbons from which the lower members of the paraffine series of hydrocarbons above propane and up to and including heptane are substantially absent. The proportion of ethyl acetate may be varied to some extent,

but it is desirable to use substantially more than 2% of ethyl acetate based on the weight of the fuel mixture.

Instead of the ethyl acetate, I may use one of a number of other esters, such for example as methyl acetate, amyl acetate, butyl acetate, or the corresponding esters of formic acid, butyric acid, propionic acid.

It will be found that motor fuels made in this manner, while containing a very large percentage of comparatively heavy hydrocarbons, can, nevertheless, be used with the greatest advantage in internal combustion engines in the same manner that light hydrocarbons have been hitherto used, and with equally advantageous results.

While I have described my invention above in detail, I wish it to be understood that many changes may be made therein without departing from the spirit thereof.

I claim:

1. A fuel comprising from 90% to 92% of a petroleum distillate heavier than 50° Bé. and an ester.

2. A fuel comprising from 90% to 92% of a petroleum distillate having a specific gravity between 30° and 50° Bé. and an ester.

3. A fuel comprising from 90% to 92% of kerosene and an ester.

4. A fuel comprising from 90% to 92% of kerosene and ethyl acetate.

5. A fuel comprising from 90% to 92% of kerosene and a volatile ester.

6. A fuel consisting of 90 to 92% of a petroleum distillate heavier than 50° Bé., and an ester.

7. A fuel consisting of 90 to 92% of kerosene, and ethyl acetate.

In testimony that I claim the foregoing, I have hereunto set my hand this 6<sup>th</sup> day of November, 1919.

MILTON C. WHITAKER.